

May 28, 1935.

G. A. KELSALL

2,002,696

MAGNETIC MATERIAL

Filed Nov. 11, 1933

4 Sheets-Sheet 1



FIG. 1



FIG. 3



INVENTOR  
G. A. KELSALL  
BY  
*J.W. Schmid*  
ATTORNEY

May 28, 1935.

G. A. KELSELL

2,002,696

MAGNETIC MATERIAL

Filed Nov. 11, 1933

4 Sheets-Sheet 2



May 28, 1935.

G. A. KELSALL

2,002,696

MAGNETIC MATERIAL

Filed Nov. 11, 1933

4 Sheets-Sheet 3

FIG. 4



INVENTOR  
G. A. KELSALL  
BY  
*John Schmid*  
ATTORNEY

May 28, 1935.

G. A. KELSALL

2,002,696

MAGNETIC MATERIAL

Filed Nov. 11, 1933

4 Sheets-Sheet 4

FIG. 6



INVENTOR  
G. A. KELSALL

BY  
J. W. Schmid  
ATTORNEY

## UNITED STATES PATENT OFFICE

2,002,696

## MAGNETIC MATERIAL

George A. Kelsall, Belleville, N. J., assignor to Bell Telephone Laboratories, Incorporated, New York, N. Y., a corporation of New York

Application November 11, 1933, Serial No. 697,576

21 Claims. (Cl. 175—21)

This invention relates to ferromagnetic materials and particularly to methods of increasing the maximum permeability of these materials.

The permeability of certain magnetic alloys, such as iron-nickel alloys and iron-nickel-cobalt alloys having special magnetic properties similar to those disclosed in U. S. Patents to G. W. Elmen 1,586,883, June 1, 1926; Elmen 1,768,237, June 24, 1930; Elmen 1,788,017, January 6, 1931; Elmen 1,715,646, June 4, 1929; and Elmen, 1,715,541, June 4, 1929, may be greatly increased by rapidly cooling these alloys through the magnetic transformation temperature range.

However, when the magnetic bodies of these alloys are large or irregular in shape and cross-section, or both, it is very difficult, if not impossible, to rapidly and uniformly cool them so that undue stresses and strains will not be set up in the bodies. These stresses and strains may reduce the permeability of the material more than the rapid cooling will increase it.

It is the object of this invention to secure a great increase in the maximum permeability of these alloys without rapidly cooling them and setting up stresses and strains in them. This is accomplished by slowly cooling the alloys in a magnetic field, the direction of which corresponds to the direction in which the high permeability is desired.

A feature of the invention resides in the discovery that the permeability of the material so treated in a direction at right angles to the direction of the magnetic field applied during the heat treatment is from 0.1 to 0.01 the permeability in the direction of the magnetic field which is applied during the heat treatment.

This invention may be more fully understood from the following descriptions of several embodiments of the invention when read with reference to the attached drawings in which:

Fig. 1 illustrates one shape of the magnetic material used and the manner in which the magnetic fields are applied to it during the heat treatment;

Fig. 2 illustrates by means of curves the effect of heat treating an iron-nickel alloy consisting of 78½% nickel and 21½% iron in accordance with this invention;

Fig. 3 illustrates the effect of the different values of field strength applied to the same alloy during heat treatment;

Fig. 4 illustrates by means of a set of curves the effect of various manners, temperatures and time durations of applying magnetic fields to the same alloy;

Fig. 5 shows several curves which illustrate the effect of various magnetic field strengths applied to an iron-nickel-cobalt alloy comprising 45% nickel, 30% iron and 25% cobalt during the heat treatment; and

Fig. 6 illustrates the effect on the permeability of various heat treatments at 725° C. and of applying the magnetic field in different directions during the heat treatment of specimens of iron-nickel-cobalt comprising 45% nickel, 30% iron and 25% cobalt.

It is to be understood that these descriptions as applied to specific alloys are to illustrate the principles and features of this invention so that it may be more clearly and fully understood but that they are not to restrict, in any way, the scope of the invention as recited in the appended claims.

Referring now to Fig. 1, 1 represents a furnace in which a core of magnetic material 2 is to be heat treated. The furnace may be of any suitable construction and heated in any convenient manner. For example, a furnace similar to that disclosed by G. A. Kelsall in an article "Magnetic testing furnace for toroidal cores" published in the July 1929 number of the Journal of the Optical Society of America and Review of Scientific Instruments, volume 19, pages 47 to 49, was used to perform some of the heat treatments to be described. In the method shown in Fig. 1, insulated windings 7 are wound on core 2 in any convenient manner, preferably insulated with asbestos or other heat resisting insulation material. Two wires are welded to opposite sides of the magnetic core 2 at 3 and 4 and are connected to a source of electrical energy 6 through a switch 5. When switch 5 is closed current will flow through both sides of the toroidal ring 2 of magnetic material and create a magnetic field within said material which will decrease from the surface of said ring to the center and will be in a direction similar to that of the wire with which coils 7 are wound. A detailed description of the magnetic field created in this manner may be found in

"Principles of Electrical Engineering" by Timbie and Bush, published by John Wiley and Sons, on pages 199 to 202 of the first edition. By connecting a source of electrical energy, not shown, to terminals 8 of winding 7, an electromagnetic field will be created within the toroidal ring 2 of magnetic material, the direction of which will be around the ring. Thus, the direction of these two fields will be substantially at right angles to each other in the magnetic material of ring 2. It is to be understood that these two fields at right

angles to each other may be obtained in any other suitable manner. If it is desired winding 7 may also be used to measure the permeability and other magnetic properties of the magnetic core 5 2 during the heat treatment.

In one experiment a ring of tape of an alloy consisting of 78½% nickel and 21½% iron which had been previously heated to above 900° C. and slowly cooled and then reheated to about 600° C. 10 and rapidly cooled by being placed upon a copper plate in accordance with the double heat treatment described in the above identified patents was heated from room temperature to above 600° C. in the manner illustrated by curve 1 of Fig. 2. 15 The temperatures of the ring are plotted as the abscissas and the time as the ordinates. It should be noted that the time scale is on the right hand side of the curve sheet and starts at the top of the sheet. Curve 2 shows the corresponding 20 permeability for a field strength of .085 gauss. This is approximately the magnetizing force for which this alloy has maximum permeability after the double heat treatment. As the temperature increases the permeability decreases to a low 25 value at a temperature slightly below 600° C. where the material becomes non-magnetic. If now the ring were slowly cooled at a rate as illustrated by curve 3 in the absence of any magnetic field the permeability on arrival at room 30 temperature would have been about 20,000 as illustrated at point X on Fig. 2. When, however, the ring was cooled in a magnetic field of .085 gauss the permeability followed curve 4 so 35 that it is higher on arrival at room temperature than after the double heat treatment. The permeability then decreased as the material was cooled to a low temperature but again increased as illustrated by curve 5 as the temperature slowly 40 rose along curve 5 to normal room temperature. It should be noted that the origin of the time scale has been shifted and the scale reduced for the low temperature treatment as illustrated by curve 5. Curve 6 shows the relation between the 45 permeability and the magnetizing force before the specimen was subjected to this heat treatment in a magnetic field, while curve 8 shows the same relation after the specimen has been heat treated in a magnetic field as described.

In addition it should be noted that since there 50 is a temperature above which the specimen becomes non-magnetic (hereinafter called the non-magnetic temperature) and also that the previous magnetic history of the specimen may be cancelled or erased by heating the specimen above this 55 temperature.

The curve in Fig. 3 shows the relation between the maximum permeability of the material and the strength of the magnetic field which is applied to it during the heat treatment. In these 60 tests an alloy consisting of 78½% nickel and 21½% iron after having been mechanically worked to its final form, which in this case is a tape wound to form a ring, is heated to a high 65 temperature above 900° C., preferably say 1000° to 1100° C., and then slowly cooled to relieve internal stresses and strains within the material. It was then reheated to above the non-magnetic 70 temperature of the material and the magnetic field of the various values applied and then the material was slowly cooled while in this magnetic field. If it is desired or convenient, this heat treatment may be made continuously with the same results by first heating the material to a 75 high temperature above say 900° C. and then

slowly cooling it in a magnetic field which may be applied at any temperature above the non-magnetic temperature of the material. However, since it is difficult to apply the magnetic field at the higher temperatures the double treatment is preferred.

As illustrated in the following Table I showing final values of initial permeability ( $\mu_0$ ) and maximum permeability ( $\mu_m$ ) either an alternating or a direct current field may be employed 10 during the heat treatment as there appears to be very little difference between these two different types of magnetic fields insofar as they effect the maximum permeability of the specimen. An alloy consisting of 78½% nickel and 21½% iron 15 was used to secure the data recorded in this table. Effective values of alternating current magnetizing force used during cooling are given.

Table I

| $\mu_0$ | $\mu_m$ | Magnetizing force in oersteds used on cooling from 600° C. |
|---------|---------|------------------------------------------------------------|
| 3150    | 14300   | 0                                                          |
| 2700    | 46500   | .10 A.-C.                                                  |
| 2100    | 64100   | .20 A.-C.                                                  |
| 2800    | 81750   | .40 A.-C.                                                  |
| 2400    | 95300   | .80 A.-C.                                                  |
| 3700    | 100500  | 1.47 A.-C.                                                 |
| 4000    | 100600  | 2.96 A.-C.                                                 |
| 3000    | 98500   | 10.35 A.-C.                                                |
| 2900    | 100500  | 2.96 D.-C.                                                 |
| 2400    | 98200   | 1.00 D.-C.                                                 |
| 2000    | 68900   | .20 D.-C.                                                  |

The curves of Fig. 4 show the effect of various 35 manners of cooling from different temperatures when an alloy consisting of 78½% nickel and 21½% iron is heat treated in a magnetic field.

In order to simplify the description of these 40 curves the first portion of the heat treatment which is slowly cooling the material from a high temperature of say 1000° to 1100° C. to room temperature to remove the stresses and strains due to the mechanical working of the specimen will be omitted, but it is to be understood that this treatment is to precede all the heat treatments described and represented by the various curves in this figure. Of course, as pointed out before, the two heat treatments may be combined if it is desired by slowly cooling from the high temperature to a temperature at which the special treatment is applied.

Point 1 shows the maximum permeability of a 45 double heat treated specimen of an alloy of 78½% nickel and 21½% iron as disclosed in the above mentioned patents in which the specimen was first slowly cooled from a temperature above 900° C., say 1000 to 1100° C., to room temperature and then reheated to 600° C. and rapidly cooled to room temperature by being placed upon a 50 copper plate.

Point 2 represents the maximum permeability 55 of the same specimen as represented by point 1 after the specimen has been heated and maintained at 400° C. for one hour. This shows that this treatment reduces the maximum permeability of the specimen by about one-third.

Curve 3 was obtained in the following manner. A specimen slowly cooled from 1100° C. in the 60 form of a ring of tape of an alloy of 78½% nickel and 21½% iron was heated to above 600° C. and then slowly cooled to 575° C. A magnetic field was then applied to the ring in which it was slowly cooled to room temperature. The 65 maximum permeability was then measured and 70

5

20

25

30

45

50

55

60

65

70

75

point 22 of curve 3 obtained. The ring was again heated to above 600° C. to cancel the previous treatment and then slowly cooled to say 550° C. A magnetic field was then applied and the ring 5 cooled to room temperature in this magnetic field. The permeability was again measured which gave point 21. In a similar manner other points were obtained by heating the ring above 600° C. and then slowly cooling it to a lower 10 temperature, hereinafter called the indicated temperature, at which time a magnetic field is applied and the ring further slowly cooled to room temperature while in this magnetic field. Then the maximum permeability was measured and 15 curve 3 plotted and drawn. The cooling rate for the points on this curve was such that it required forty-five minutes to cool the ring from 600° C. to 200° C. While it is not necessary to employ the same ring for all the points on a 20 curve it is desirable to do so since it eliminates the variations between the different rings. It is necessary that the stress and strains have been removed by slowly cooling the specimens from a high temperature and that other previous heat 25 treatments and magnetic effects have been cancelled by heating the material above its non-magnetic temperature.

Curve 4 shows the maximum permeability of another specimen after it was heated to 600° C. 30 and then slowly cooled to the indicated temperature at which time the magnetic field was applied, and then the specimen was maintained at this temperature in the magnetic field for one hour after which time it was slowly cooled 35 in the magnetic field to room temperature in such a manner that the specimen would have been cooled from 600° C. to 200° C. in forty-five minutes. It should be noted that when the specimen was cooled to some temperature below 400° 40 before the magnetic field was applied, the permeability is the same for both treatments represented by curves 3 and 4 as illustrated by the portion 45 of these curves and is of a comparatively low value. This is probably due to the fact that the cooling rate of these specimens from 600 to some temperature below 400° C. was the same. This fact also indicates that some phenomenon takes place between the temperatures of 600 and 400° C. for this particular alloy 50 which greatly influences the maximum magnetic permeability of the specimen. This temperature region from a temperature near or above the magnetic transformation temperature to a lower temperature of approximately 400° C. will be 55 called the magnetic transformation temperature region in what follows hereinafter.

The heat treatment which produced the resultant maximum permeability as shown by curve 5 was as follows: The slowly cooled specimen 60 was placed in a hot furnace at the temperature indicated and allowed to remain there for fifteen minutes. This provided adequate time to allow the specimen to acquire the temperature of the furnace. A magnetic field was then applied to the specimen which was then slowly cooled in such a manner that it would require one hour and thirty-five minutes to cool it from 600° C. to 200° C.

To secure the maximum permeability as shown 65 by curve 6 the specimen was placed in the furnace at the indicated temperature and allowed to remain there for fifteen minutes. The magnetic field was applied at the same time the specimen was introduced into the furnace so that the 70 field was acting upon the specimen during the

heating of the specimen. The specimen was then allowed to slowly cool in the magnetic field at the same rate which was used in obtaining curve 5.

For curve 7 a specimen was raised to 600° C. 5 and then slowly cooled. On arriving at the indicated temperature the magnetic field was applied to the specimen and it was maintained at this temperature in the magnetic field for five hours and then slowly cooled to room temperature at a cooling rate such that it required one hour and thirty-five minutes to cool the specimen from 600° to 200°. The permeability of the specimen as treated for curves 5, 6 and 7 approaches 10 the same value when the magnetic field is applied at 375° C. or below and, as illustrated by the portion 15 11 of these curves, is of a lower value than that of curve 10. This is due to the slower cooling rate which is about half that employed when the specimen was treated for curves 3 and 4 so 20 that it required twice as long to cool the specimen in this case as it did for curves 3 and 4.

For obtaining curve 8 several specimens from the same lot of material of an alloy of 78½% nickel and 21½% iron were used. They were all 25 slowly cooled from a high temperature to remove the stresses and strains due to working. They were then reheated to above 600° C. where a magnetic field was applied and then they were slowly cooled. Each specimen was cooled to a different 30 temperature and maintained at these respective temperatures in the magnetic field for five hours after which time they were slowly cooled to room temperature. The cooling rate was such that it would require thirty-one minutes to cool the 35 specimens from 600° C. to 200° C. The permeabilities were then measured and plotted as a function of the temperature at which the specimens remained for five hours.

Curve 9 shows the result of maintaining the 40 specimens as heat treated for curve 8 at 400° C. for one hour. This shows a much less decrease in permeability by baking for one hour at 400° C. while not in a magnetic field than that shown by the ordinary double heat treated specimen as 45 illustrated by the difference between points 1 and 2. Thus the permeability of the specimen heat treated in a magnetic field as for example in accordance with heat treatment for curve 8 is believed to be much more stable and permanent 50 and less subject to change with time and temperature than it is for the ordinary double heat treatment now in use.

The curves in Figs. 5 and 6 show the permeabilities of an iron-nickel-cobalt alloy comprising 55 45% nickel, 30% iron and 25% cobalt as treated in accordance with this invention. It should be noted that the curves of Fig. 6 are plotted on logarithmic scales so that the range in value of the permeability is greater than it 60 appears from these curves. Curve 1 in Fig. 5 shows the effect of various field strengths used during cooling upon initial permeability of the sample as it was taken from the heat treating furnace at room temperature. For curve 2 the 65 sample has been demagnetized. Curve 3 shows the maximum permeability of the sample as it came from the furnace for various magnetic field strengths used during the heat treatment and for curve 4 the specimen has again been demagnetized. 70

Curve 1 of Fig. 6 shows the relation between the permeability and the magnetizing force of a specimen of an iron-nickel-cobalt alloy consisting of 45% nickel, 30% iron and 25% cobalt in 75

the form of a solid ring after it has been heated to 1100° C. and maintained at this temperature for one hour and then slowly cooled. In curve 2 the specimen was then heated to 725°, which is 5 slightly above the non-magnetic temperature of this alloy, for fifteen minutes and slowly cooled. In both of these cases no magnetic field was applied to the specimen during the heat treatment. For curve 3 after the specimen had been cooled 10 from 1100° C. it was again heated to 725° C. for fifteen minutes and slowly cooled with the cross magnetic field applied during cooling by sending an electrical current through the specimen as illustrated in Fig. 1. It is to be noted that this 15 somewhat increases the permeability at low magnetizing forces but that the permeability still remains fairly constant to rather high values of H. For curve 4 the specimen was heated to 725° C., which is slightly above the non-magnetic temperature for this alloy, for fifteen minutes after it had previously been slowly cooled from 1100° C. A direct current magnetic field of 24 gauss was then applied and the specimen slowly cooled. This field was applied circumferentially in the 20 same direction in which the permeability was measured. For curve 5 the specimen was again heated, after cooling from 1100° C., to 725° C. for ten minutes and then rapidly cooled by dropping it into water with no magnetic force applied. 25 For curve 6 the specimen was similarly treated excepting that it was quenched in oil instead of water. For curve 7 two layers of 3 mil metallic tape were wrapped about the specimen in order to prevent too rapid a cooling of the surface so 30 that excessive strains would not be set up within the specimen.

From these curves it is evident that this material behaved similar to the iron-nickel alloy consisting of 78½% nickel and 21½% iron in that 40 rapidly cooling it through the magnetic transformation temperature region, in this case from between approximately 725 and 400° C., produces a marked increase in the maximum permeability of the specimen; and, also, that applying a magnetic field while slowly cooling the specimen through this temperature region very greatly increases the maximum permeability of the material. In addition, from curves 3 and 4, it is quite evident that there is a difference in the 45 maximum permeability of more than 60 to 1, and for certain values of field strength there is a difference of more than 100 to 1 between the permeability in the direction which coincides with the direction of the magnetic field employed during the heat treatment and the permeability at 50 right angles to that direction. By the use of such a material having these properties it is quite evident that the stray magnetic flux surrounding magnetic cores can be reduced since 55 the flux would tend to follow the direction of the magnetic field applied during the heat treatment. A further advantage of the iron-nickel-cobalt alloys as heat treated in a magnetic field is that the maximum permeability occurs for 60 relatively high values of flux densities so that for a range of flux density from 12,000 to 14,500 the permeability is higher than that for any other substance known today.

In later tests it was found unnecessary in some 70 cases to heat alloys of iron, nickel and cobalt to over 900° C. and slowly cool them to remove internal stresses and strains. It was found that a temperature as low as 700° C. was sufficient to remove the internal strains. This is especially 75 true if it is maintained at this temperature for

some time. In these cases it is necessary to heat specimens of these alloys to this temperature only, apply the magnetic field and slowly cool them.

The following Table II shows the results of 5 treating various magnetic alloys in accordance with this invention.

Table II

| Material        | $\mu_0$           | $\mu_m$              | H in oersteds used on cooling | Temperature °C.   |
|-----------------|-------------------|----------------------|-------------------------------|-------------------|
| Nickel          | 230<br>220        | 1287<br>1328         | 0<br>26.5                     | 460<br>460 15     |
| 45% nickel      | 3100              | 11000                | 0                             | 500               |
| 55% iron        | 3400              | 11470                | 6.65                          | 500               |
| 70% nickel      | 1130              | 7290                 | 0                             | 625               |
| 30% iron        | 2250<br>3300      | 44300<br>44520       | 6<br>0                        | 625               |
| 78.5% nickel    | 7000              | 26800                | 0                             | 600               |
| 3.8% chromium   | 7000              | 27950                | 6.0                           | 600               |
| 17.7% iron      |                   |                      |                               |                   |
| 78.5% nickel    | 9850              | 46600                | 0                             | 480               |
| 3.8% molybdenum | 9650              | 52900                | 5.4                           | 480               |
| 17.7% iron      |                   |                      |                               | 25                |
| 50% iron        | 2600              | 3980                 |                               |                   |
| 50% cobalt      | 540               | 6750                 | 27                            | 1025              |
| Armeo           | 2160              | 26950                |                               |                   |
| Iron            | 100               | 8600                 | 25                            | 800               |
| Silicon steel   | 340<br>300<br>240 | 5820<br>5800<br>7880 | 0<br>30 A. C.<br>30 D. C.     | 810<br>810<br>810 |

<sup>1</sup> For regular double treatment.

<sup>2</sup> After vacuum annealing at 1000°.

<sup>3</sup> After vacuum annealing at 925°.

35 This table shows that those alloys which respond to rapid cooling through the magnetic transformation temperature region also exhibit a marked increase in maximum permeability when slowly cooled in a magnetic field through its magnetic transformation temperature region.

40 By treating magnetic alloys in accordance with this invention the permeability in many cases exceeds that which may be obtained by the usual double heat treatment and in addition the alloy seems to be more stable magnetically. Furthermore, this method may be applied to all types of 45 magnetic bodies of various shapes and cross-sections. It is, moreover, impossible to rapidly and uniformly cool some large or irregularly shaped magnetic sections of either solid or laminated constructions so as to secure a great increase in the maximum permeability. This is due to the fact that the rapid cooling cannot be uniformly controlled throughout the section so that 50 various portions of the section which may be of different shapes and cross-sections will be cooled at considerably different rates. This may develop large stresses and strains within the section which may reduce the permeability more than the rapid 55 cooling increases it. For example, a large cylindrical casting of an alloy of 78½% nickel and 21½% iron was double heat treated by quenching and the maximum of permeability obtained was about 9000 while by heat treating it in a magnetic field in accordance with this invention by slowly cooling it from 600° C. in the magnetic field, a maximum permeability of 111,000 was obtained.

60 In addition, the permeability for high values of induction of alloys having high saturation values of induction when heat treated in a magnetic field in accordance with this invention is in excess of the permeabilities at these high values of induction of any magnetic material known today.

35

40

50

55

60

65

70

75

It should also be noted that while no figures have been given relating to the hysteresis, magnetic alloys treated in accordance with this invention have the hysteresis loss reduced in a manner similar to the reduction secured by the double heat treatment in which the alloy is rapidly cooled through the magnetic transformation temperature. This method of heat treatment possesses the further advantage of tending to reduce stray magnetic flux leakages from cores heat treated in this manner since the permeability in the desired direction may be made many times greater than the permeability at right angles thereto. This would be an advantage in relay structures and other types of magnetic apparatus in which it is desired to reduce or limit the value of the stray magnetic flux.

This treatment also produces more uniform permeability throughout the cross-section of specimens.

What is claimed is:

1. A method of increasing the magnetic permeability of irregularly shaped magnetic bodies made of magnetic alloys, the permeability of which is increased by rapidly cooling them through the magnetic transformation temperature region, characterized in that said magnetic bodies are slowly cooled through the magnetic transformation region in a magnetic field directed in the direction in which the high permeability is desired.

2. A method of increasing the magnetic permeability of ferro-magnetic materials, the permeability of which is increased by rapidly cooling them through the magnetic transformation temperature region, which comprises cooling the material in a magnetic field from a temperature above the magnetic transformation temperature region of the material.

3. A method of increasing the maximum magnetic permeability of magnetic bodies of irregular shapes and cross-sections of magnetic alloys, the maximum permeability of which is increased by rapidly cooling them through the regions of the magnetic transformation temperatures which comprises slowly cooling the bodies from a high temperature and then reheating and slowly cooling the bodies in a magnetic field from a temperature below the non-magnetic temperature of the material.

4. A method of increasing the permeability of magnetic bodies of large cross-sections, the permeability of which is increased by rapidly cooling the magnetic material of said bodies through the region of the magnetic transformation temperatures which comprises slowly cooling the bodies from a high temperature through the magnetic transformation temperature region while subjected to a magnetic field.

5. A method of heat treating magnetic alloy which comprises slowly cooling the alloy from a temperature above 900° C., reheating it to a temperature above non-magnetic temperature and cooling it through the magnetic transformation temperature region in a magnetic field.

6. A method of heat treating magnetic alloy which comprises heating the alloy to a temperature above 900° C., slowly cooling the alloy to a temperature above non-magnetic temperatures of the alloy, applying a magnetic field to the alloy and cooling the alloy through the magnetic transformation temperature region in said magnetic field.

7. A method of heat treating magnetic alloy which comprises slowly cooling the alloy from a temperature above 900° C., reheating it to a tem-

perature within the magnetic transformation temperature region but which is below the non-magnetic temperature of the alloy, in a magnetic field and slowly cooling the alloy in said magnetic field.

8. A method of heat treating magnetic alloys which comprises slowly cooling the alloy from a temperature above 900° C. to a temperature below non-magnetic temperature but within magnetic transformation temperature range, applying a magnetic field to the alloy and cooling the alloy in said magnetic field.

9. A method of heat treating magnetic alloys which comprises slowly cooling the alloys from a temperature above 900° C., reheating it to a temperature within the magnetic transformation temperature region, applying the magnetic field to said alloy, maintaining said alloy at said temperature in said magnetic field for a time and cooling said alloy in said magnetic field.

10. A method of heat treating magnetic alloys which comprises slowly cooling the alloys from above 900° C. to a temperature within the magnetic transformation temperature region, applying a magnetic field to said alloy and maintaining said alloy in said magnetic field for a specified time and then cooling the alloy in said magnetic field.

11. A method of increasing the maximum permeability of large magnetic bodies of alloys comprising nickel and iron which comprises slowly cooling the alloy from a temperature above 900° C., reheating the bodies to a temperature within the magnetic transformation temperature region and cooling said alloy in a magnetic field.

12. A method of increasing the maximum permeability of alloys comprising nickel and iron which comprises slowly cooling the alloy from a temperature above 900° C., reheating the alloy in a magnetic field to a temperature within the magnetic transformation region, maintaining the alloy at said temperature in the magnetic field for a specified time and then cooling the alloy in said magnetic field.

13. A method of increasing the maximum permeability of large magnetic bodies of irregular cross-sections of magnetic alloys comprising nickel and iron which comprises slowly cooling the alloy from a temperature above 900° C. to a temperature within the magnetic transformation region of said alloy, applying a magnetic field to said magnetic bodies and cooling said magnetic sections in said magnetic field.

14. A method of heat treating magnetic bodies of large and irregular cross-sections of magnetic alloys comprising nickel and iron which comprises cooling said magnetic sections from a temperature above 900° C. to a temperature within the magnetic transformation temperature region, applying a magnetic field to said bodies, maintaining said bodies at said temperature in the magnetic field for a time, and slowly cooling the bodies in said magnetic field.

15. A method of heat treating large magnetic bodies of magnetic alloys comprising iron, nickel and cobalt which comprises slowly cooling said bodies from a temperature above 900° C., reheating it to a temperature within the magnetic transformation temperature region and cooling it in a magnetic field.

16. A method of increasing the maximum permeability of large irregularly shaped magnetic bodies of magnetic alloys comprising nickel, iron and cobalt, which comprises slowly cooling the alloy from a temperature above 900° C., reheat-

ing the alloy to a temperature within the magnetic transformation temperature region, maintaining the bodies at said temperature and in a magnetic field for a short time period and slowly cooling the sections in the magnetic field.

17. A method of heat treating magnetic alloys comprising nickel, iron and cobalt to secure a high maximum permeability in one direction to said alloy and a relatively low permeability in a direction at right angles thereto, which comprises slowly cooling said alloy from a temperature above 900° C. to room temperature, reheating said alloy in a magnetic field in a direction in which the high permeability is desired to a temperature within the magnetic transformation temperature region of said alloy, and slowly cooling said alloy in said magnetic field.

18. A method of reducing magnetic leakage from the cores of electromagnetic apparatus by heat treating said cores to secure a high permeability in the direction of the desired flux and a low permeability in the direction of the leakage flux, which comprises slowly cooling said

cores from a temperature above 900° C. to room temperature, reheating said cores in a magnetic field to a temperature within the magnetic transformation temperature region in a magnetic field and slowly cooling said cores to room temperature in said magnetic field.

19. A method of treating magnetic alloy of iron, nickel, and cobalt which comprises heating said alloy above its non-magnetic temperature, applying a magnetic field to said alloy, and cooling said alloy in said field.

20. A method of increasing the permeability of large irregularly shaped magnetic sections of alloys comprising iron, nickel, and cobalt which comprises heating said sections to above 725° C., applying a magnetic field, and cooling said sections in said magnetic field.

21. A magnetic material having a permeability to magnetic fields directed in one direction in the material which is over five times the permeability of the material to magnetic fields directed in other directions in the material.

GEORGE A. KELSALL.